# EUROPEAN PATENT SPECIFICATION

(11) **EP 2 029 455 B1**
(45) Date of publication and mention of the grant of the patent: **11.03.2015**
(21) Application number: 07766758.2
(22) Date of filing: 14.06.2007
(51) Int. Cl.: B65D 83/14

(54) **NON-ROUND PLASTIC PRESSURIZED DISPENSER**
NICHT RUNDER DRUCKSPENDER AUS KUNSTSTOFF
DISTRIBUTEUR SOUS PRESSION PLASTIQUE NON ROND

(30) Priority: 16.06.2006 US 454806
(43) Date of publication of application: 04.03.2009
(73) Proprietor: THE PROCTER & GAMBLE COMPANY, Cincinnati, OH 45202 (US)
(72) Inventor: ALTONEN, Gene, Michael, West Chester, OH 45069 (US); DODD, Michael, Thomas, Florence, KY 41042 (US); KHAN, Ayub, Ibrahim, Cincinnati, OH 45249 (US); MURDOCK, William, Dale, Cheviot, OH 45211 (US); QUIRAM, Daniel, Jonathan, Midlothian, VA 23114 (US)
(74) Representative: Holmes, Rosalind
(86) International application number: PCT/IB2007/052276
(87) International publication number: WO 2007/144847

(56) References cited:
- EP-A- 0 399 793
- EP-A- 0 664 201
- US-A- 5 071 015
- US-A1- 2005 123 494
- US-A1- 2005 242 101
- US-A1- 2006 060 554

## Description

### FIELD OF THE INVENTION

The present invention relates to a plastic pressurized package that is substantially non-round in cross-section and capable of being exposed to and containing a variety of personal care products, has high impact resistance, chemical resistance, and thermal stability.

### BACKGROUND OF THE INVENTION

Pressurized or aerosol antiperspirant products have been marketed for many years. These products are typically packaged in metal cans or glass containers. For many products, it is advantageous for the package to be clear to permit the contents to be viewed by a user. While glass provides this option, it is typically expensive and can be very fragile when dropped. A much less common material used to form a pressurized package is plastic. Plastics, such as grades of amorphous polyamide and polyester, provide a clear container for viewing purposes and have the added advantages of being less fragile and more economical to produce versus glass. Also, unlike metal aerosol containers, plastic aerosols can be formed into a variety of shapes and cross-sections. Most existing plastic aerosol packages, however, are limited to round cross-sections in order to ensure that certain performance and safety requirements are met as required prior to distribution and use. Because plastic pressurized containers are also known to have several disadvantages, standard test procedures, such as British Standard 5597:1991, provides a means for ensuring the package is safe under normal usage conditions.

A common disadvantage to a pressurized plastic container includes the fact that existing plastic pressurized containers are typically comprised of polyester terephthalate (PET) which has a thermal softening point of about 60-66°C. This is undesirable since it is possible, in fact likely, that a plastic container will be exposed to temperatures above 60°C, or even higher than about 70°C, particularly inside an automobile on a hot summer day. While certain plastic materials, such as polyester naphthalate (PEN), polyarylate (PAR), and blends of polyesters have been used by some manufacturers to increase the thermal softening point to above 90°C, these materials are very expensive relative to PET. Also, PEN and PAR have a yellow hue and thus, are not well suited for certain applications since they have relatively poor optical clarity. Thus, there is a need for an affordable material option that provides plastic pressurized containers with structural integrity at temperatures above 60°C or even above 70°C while providing good optical clarity.

Another disadvantage is that existing plastic pressurized containers generally cannot survive drop impacts of greater than about 1.83 m (6 feet). While this is generally considered an acceptable level of impact resistance by those skilled in the art, it is the intent of the present invention to provide a container with even greater resistance to impact, since in certain circumstances it is possible that the container could be exposed to impact stresses exceeding a 6 foot drop impact, such as when dropped from the top shelf in a retail store.

Further, many existing plastic pressurized containers are susceptible to degradation by many solvents commonly used in consumer products. When the plastic material used to form a plastic pressurized container is degraded by a solvent, the ability of the container to contain pressure, resist impact, and to provide good optical clarity can be diminished. Providing a plastic material that resists degradation caused by common solvents results in a plastic pressurized container that is better suited to contain a large range of consumer products and thus, has greater commercial value. The present invention, therefore, provides the advantage of making a more economical, structurally sound and aesthetically-pleasing package that is capable of containing a wide range of consumer products.

A plastic pressurized package according to the preamble of claim 1 is for instance known from document US-A-2006/0060 554.

### SUMMARY OF THE INVENTION

The present invention relates to a plastic pressurized package as defined in claim 1.

### DETAILED DESCRIPTION OF THE INVENTION

The present invention relates to a plastic pressurized package capable of being exposed to and containing a variety of personal care products, has high impact resistance, chemical resistance and thermal stability. By combining two or more materials that form the walls of the package, the present invention provides substantial advantages in achieving an ideal combination of physical and chemical properties that are not typical in a glass and metal aerosol packages.

While the specification concludes with the claims particularly pointing and distinctly claiming the invention, it is believed that the present invention will be better understood from the following description.

Except where specific examples of actual measured values are presented, numerical values referred to herein should be considered to be qualified by the word "about".

As used herein, "comprising" means that other steps which do not affect the end result can be added. This term encompasses the terms "consisting of" and "consisting essentially of". The methods/processes of the present invention can comprise, consist of, and consist essentially of the essential elements and limitations of the invention described herein, as well as any of the additional or optional components, steps, or limitations described herein.

All percentages, parts and ratios are based upon the total weight of the compositions of the present invention, unless otherwise specified. All such weights as they pertain to listed ingredients are based on the active level and, therefore, do not include solvents or by-products that may be included in commercially available materials, unless otherwise specified. The term "weight percent" may be denoted as "wt.%" herein.

It is also herein contemplated that the present invention may be practiced with many consumer products including, but not limited to, antiperspirants, deodorants, hair products, household products, cooking sprays, beverages, perfumes, shaving creams/gels, or drug products.

The term "non-round" is defined herein as the shape of the pressurized plastic dispenser of the present invention wherein the shape, when viewed in any cross-section, is substantially not geometrically round and is capable of substantially maintaining said shape when subjected to the pressure exerted by the contents within the plastic package of the present invention. For example, shapes of the present invention, when viewed in cross-section, may include, but are not limited to, square, rectangle, oval, star, heart, diamond, polygons, trapezoid, rhombus, triangle, and the like.

The term "plastic" is defined herein as any polymeric material that is capable of being shaped or molded, with or without the application of heat. Usually plastics are a homo-polymer or co-polymer of high molecular weight. Plastics fitting this definition include, but are not limited to, polyolefins, polyesters, nylon, vinyl, acrylic, polycarbonates, polystyrene, and polyurethane.

The term "clear" is defined herein as having the property of transmitting light without appreciable scattering so that bodies lying behind are perceivable. One acceptable test method for determining whether a product is clear is to attempt to read a series of words placed immediately behind the package. The words being printed in black color, 14 point Times New Roman font, printed on a white sheet of paper with the printed side of the paper attached to the back of the package. The word and/or letters must be visible and/or readable from the front of the package by an individual of reasonable eyesight and positioned directly in front of the package

The term "optical clarity" is defined herein as the ability of a material to transmit light through the material. Optical clarity is characterized by both the luminous transmittance of light through a material and also by its haze value (as defined in ASTM method D1003). The approximate haze level of a container can be determined by comparing the container to flat test samples having known haze values. The haze level of the container can be approximated by finding a test sample with a slightly lower haze value, and a sample having a slightly higher haze value. The approximate haze value of the container is based on the value found between the value of the two test samples. Haze values may be determined as described herein.

The term "tinted" is defined herein as the practice of adding a low level of pigment or dye into a material for the purpose of imparting a level of opacity, color, or opacity and color into the material.

The term "plastic package" refers to the container vessel of the pressurized package being made substantially of plastic. The sealing valve and actuator of the package may or may not necessarily be made substantially of plastic.

The term "pressurized plastic dispenser" or "pressurized plastic package" is defined herein as a container with fluid contents such as propellants, wherein the fluid contents have a pressure of at least 103.4 kPa (15 psi), at least about 206.8 kPa (30 psi), at least about 310.2 kPa (45 psi) or at least about 413.6 kPa (60 psi) greater than atmospheric pressure at 25°C but no more than about 956.1 kPa (140 psi), no more than about 896.1 kPa (130 psi), no more than about 758.3 kPa (110 psi) or no more than about 620.4 kPa (90 psi) greater than atmospheric pressure at 25°C. The pressurized plastic package of the present invention is able to contain and dispense fluids with the above-mentioned pressure limitations while substantially maintaining a non-round cross-section shape.

The term "deform" or "deformation" describes the change in shape or form in a material caused by any type of stress, force or degradation. If a material exhibits excessive deformation, the material may exhibit a mode of failure such that the material breaks, expands or ruptures due to its inability to resist high temperatures, impact stresses, and contents of certain fluids or gases, particularly pressurized fluids.

The term "resistant to chemicals" or "chemical resistance" describes an opposition to certain chemicals that would normally degrade and/or crack the plastic material. These "certain chemicals" may be those commonly known as household solvents or solvents commonly used in consumer products. Such chemicals include, but are not limited to, ethanol, acetone, glycol, waxes, oils, hydrocarbon-based silicones, and the like. Resistance to common household solvents ensures that the container does not leak or rupture when exposed to certain liquids. Chemical resistance may be determined and measured as described herein.

The term "thermal resistance" refers herein to a pressurized container that shows no visible sign of deformation after exposure to high temperatures such as 58°C for about 2 minutes, 60°C for about 2 minutes, 65°C for about 2 minutes or 70°C for about 2 minutes.

The terms "crystalline" or "crystallizable" polyethylene terephthalate (PET), refers herein to PET homopolymers or copolymers that are capable of forming crystalline structures on cooling from the melt, or resulting from exposure to heat (thermal induced crystalinity) or immersion in a suitable solvent (solvent induced crystalinity).

The term "non-crystallizing" or "non-crystallizable" polyethylene terephthalate (PET), refers herein to PET copolymers (also called PET co-polyesters) that are substantially incapable of forming crystalline structures during cooling from the melt state or during exposure to heat (thermal induced crystalinity), or when exposed to solvents and vapors (solvent induced crystalinity).

The term "amorphous" PET, as used herein, refers to "non-crystallizing" or "non-crystallizable" polyethylene terephthalate (PET) that substantially resist the formation of crystalline structures resulting from exposure to heat (thermal induced crystalinity) or immersion in suitable solvents and vapors (solvent induced crystalinity).

As used herein, "polycarbonate (PC)" refers to polycarbonate of the types synthesized from Bisphenol A, those synthesized from alternative monomers, random copolymers, block copolymers, and blends thereof.

As used herein, "filler" includes materials included to reduce the total amount of polymer in a given space.

"Additives" refers to materials, known in the art to impart a desired property, including, but not limited to anti-stat, anti-scuff, optical brightness.

### Plastic Pressurized Package

The plastic pressurized package of the present invention exhibits particular enhanced characteristics such that it is capable of containing and being exposed to a variety of personal care products, has high impact resistance, chemical resistance and thermal stability. The plastic pressurized package is formed from a combination of at least one first and second polymer material. Combining at least a first and second material to form the parts of the package provides substantial advantages in achieving an ideal combination of physical, chemical and aesthetic characteristics that are not typical in glass and/or metal aerosol packages. Colorants, fillers and additives can be incorporated into the polymer mixture to impart desirable aesthetics, mechanical, or functional properties.

### Materials

### Combination Materials

A combination of materials including at least a first and a second material is used, wherein said first material and said second material are different. According to the invention, the first material is included at a ratio of greater than 70% in relation to the second and optional additional materials. The combination may also optionally include additional materials to the first and second material. Combination materials useful to the present invention, include the following:

### First Material

The first materials of plastic parts useful in the present invention include, polyesters, polyester copolymers, and mixtures thereof. Polyesters may be selected from the group consisting of polyethylene terephthalate (PET), polyester copolymers and mixtures thereof. Polyester copolymers are preferably selected from the group consisting of polyethylene terephthalate glycol-modified (PETG), polycyclohexanedimethanol terephthalate (PCT), polycyclohexanedimethanol terephthalate isophthalate (PCTA), polycyclohexanedimethanol terephthalate glycol (PCTG), and mixtures thereof. The polyester copolymers preferably comprise monomers selected from the group consisting of isophthalic acid (IPA), terephthalic acid (TPA), butane diol (BD), cyclohexanedimethanol (CHDM), ethylene glycol (EG), diethylene glycol (DEG) and mixtures thereof. Additional materials useful for the present invention include, but are not limited to, polypropylene (PP), cyclic polyolefin copolymer (COC), polystyrene (PS), Barex (Impact modified acrylonitrile-methyl acrylate copolymer), and styrene acrylonitrile copolymer (SAN).

Polyethylene terephthalate (PET) may be obtained in various forms depending upon how it is processed and crystallized. When rapidly cooled from the melt, PET can be obtained in a substantially amorphous non-crystalline form (APET) which is transparent. If PET is processed and cooled under controlled conditions, for example while being oriented in a blow molding or film stretching operation, a semi-crystalline form can be obtained which may still be transparent as long as the crystalline size is maintained below the wavelength of visible light such as from about 400nm to about 700nm. If PET is cooled slowly from the melt such that the crystalline structures can grow larger than the wavelength of light, it can be obtained in a semi-crystalline form which is hazy or even opaque depending upon the degree of crystallization that occurs.

Generally, the term "crystalline" or "crystallizable" PET is typically reserved for PET homopolymers, PET copolymers, or blends thereof, that are themodynamically capable of forming crystalline structures when cooled from the melt state, or exposed in the solid state to temperatures at about or above the Tg of PET (thermal induced crystallinity), or exposed to a suitable solvent or vapor (solvent induced crystallinity). The term "non-crystallizing " PET is typically reserved for PET copolymers that substantially resist the formation of crystalline structures. These "non-crystallizing" PET materials are particularly useful in the context of the current invention since these materials can be processed into thickwall containers while substantially limiting the formation of thermal induced crystalline structures. Furthermore, these "non crystallizing" PET materials substantially resist the formation of crystalline structures resulting from exposure to solvents commonly used in consumer products. Thus, these transparent materials resist the tendency to haze or become opaque when exposed to consumer products.

### Second Material

The second material of plastic parts useful in the present invention include, but are not limited to polyamides, polycarbonates, polyacrylates, polycarbonate copolymers, polyesters, polyester copolymers, and mixtures thereof. Although PCs are generally known in the art to have bad chemical tolerance and/or resistance, the present invention prefers PCs as the second material to blend with the first material. It has been discovered, contrary to the usual characteristics of PC, that when blended with the first material of the present invention, the chemical and heat resistance of the plastic parts are enhanced which contribute to the enhanced structural integrity of the plastic aerosol dispenser of the present invention. This is outside of the expected characteristics of PC because PC has very poor resistance to common solvents such as ethanol and even water. For example, a container formed from PC will rapidly haze and even crack if doused with ethanol for just a few seconds. Therefore, one would expect that blending PC with a material having better chemical resistance, such as a PET or PET copolymer, would result in a material with a lower resistance to solvents. The present invention, however, has discovered that PC can be blended with PET and PET copolymers at levels up to about 40% while providing a material with chemical resistance similar to the PET material alone. Again, realizing that PET has an undesirable thermal softening point of about 60-66°C, the blend of a polyester such as PET with PC provides an overall advantageous plastic aerosol dispenser that imparts enhanced chemical, physical and marketable characteristics that is currently absent from the art.

Polycarbonate (PC), most commonly refers to a polycarbonate plastic made from Bisphenol A, where Bisphenol A functional groups are linked together by carbonate groups to form a polymer chain. This thermoplastic material is highly transparent to visible light, has excellent mechanical properties, i.e., polycarbonate is commonly used to form "bullet proof glass, and has very good thermal resistance. Thus, PC is useful in the context of the current invention since it has outstanding impact resistance, can form a container with very good optical clarity, and can form a container that resists thermal deformation at temperatures above about 65°C or even above about 70°C. It is further understood, that polycarbonate materials can be synthesized from a variety of monomers and that polycarbonate random copolymers and block copolymers may also be well suited to provide the desired material properties for the current invention.

The plastic pressurized packages of the present invention comprise a minimum wall thickness of about 0.65 mm, about 1.0 mm, about 1.30 mm, about 1.95 mm, about 2.60 mm, or about 3.25 mm and may be of various shapes, for example round and non-round. Additionally, the pressurized plastic packages exhibit the following combined benefits, features and/or manufacturing methods.

### High Optical Clarity

Optical clarity is characterized by both the luminous transmittance of light through a material and also by its haze value (as defined in ASTM method D1003). Packages of the present invention may have a transmittance value greater than about 85% or greater than about 90%. The initial haze value may be less than about 10%, less than about 5%, or less than about 2%.

### High Impact Strength

The term "impact resistance'' or "impact strength" describes an opposition to stresses which ensures that a container does not leak or rupture when exposed to mechanical stresses such as an impact on a hard surface. Packages of the present invention will withstand without damage a drop impact from a vertical distance of at least about 1.83 m (6 feet), at least about 3.05 m (10 feet), at least about 4.27 m (14 feet), or at least about 5.49 m (18 feet).

### High Heat Deflection Temperature. (HDT)

HDT describes the temperature at which a plastic material will become deformable under an applied load such as the pressure exerted by an aerosol propellant (defined by ASTM method D648). Packages of the present invention may have a HDT of at least about 65°C, at least about 70°C, or at least about 80°C, all under an applied load of about 455.1 kPa (66 psi).

### High Chemical Resistance

Chemical resistance is the ability of a material to resist chemical or physical degradation over time due to being in contact with another chemical substance. One way to assess the chemical! resistance of a material is to determine the change in haze value of the material. Haze values may be determined by standard procedures such as ASTM D 1003. The test is performed by comparing the test specimen to certified haze value standards such as that provided by BYK-Gardner, USA, Columbia, MD.

The haze level of a test sample of the material is taken. The test sample is then exposed to a chemical substance, such as a consumer product, for a controlled time period, such as at least about 1 week, and a controlled temperature, such as 49°C. Following exposure to the chemical, the haze level is measured again. If the haze level does not change, or changes very little, then the material is said to provide excellent chemical resistance to the chemical substance. If there is a substantial increase in the haze level, the material is said to have poor chemical resistance to the chemical. The change in haze level is equal to the absolute value of the initial haze value minus the final haze value, and is designated as "Δ_{haze"}. Table 1 below provides guidelines for what one could consider excellent, good, fair, or poor chemical resistance of the pressurized plastic containers of the present invention stored for 1 week at 49°C.

**Table 1**

| **Chemical Resistance** | **Δ_{haze}** |
|---|---|
| Excellent | < about 10% |
| Very Good | about 10% - about 20% |
| Good | about 20% - about 30% |
| Fair | about 30% - about 40% |
| Poor | > about 40% |

An additional method to assess the chemical resistance of a pressurized plastic container is to fill several pressurized plastic containers with a chemical substance, such as a pressurized consumer product. The filled containers are then conditioned for a controlled time period and at a controlled temperature. Elevated temperatures can be used to accelerate the rate that a chemical interaction will occur. After conditioning, the container can then be evaluated to determine if the container has been degraded by the chemical substance using technical tests such as: dropping the filled containers on a hard surface (concrete or steel) from a certain height, for example, about 1.83 m (6 feet); visually examining the packages for evidence of degradation such as an increase in haze (Δ_{haze}) or a change in color; and resistance to thermal deformation. The table below provides an example of a typical test procedure.

**Table 2**

| **Preparation Steps** | | **Description** | **Success Criteria** |
|---|---|---|---|
| 1 | Container Measurement | Measure reference dimensions of each container to be placed in testing (60 total containers). | NA |
| 2 | Container Preparation | Fill containers with consumer product to 80% capacity. Consumer product includes concentrate and propellant. | NA |
| 3 | Sample Conditioning | Condition 10 filled containers at: about 40°C for 12 weeks; about 21°C fo 26 weeks. | NA |
| | | | |

| **Testing Steps** | | **Description** | **Success Criteria** |
|---|---|---|---|
| 4 | Visual | Visually inspect packages for | <20% Δ_{haze}, and more |
| | Evaluation | change in haze level, discoloration, or other evidence of chemical interaction. | preferably <10% Δ_{haze}; No noticeable discoloration. |
| 5 | Impact Resistance | Drop packages from a height of 1.83 m (6 feet), three times, in random orientation. | No distortion, no cracks, no leaks. |
| 6 | Thermal Resistance | Bring package & contents to a temperature of about 58°C for about 2 minutes, | No visible and/or permanent distortion, no leaks, no cracks. |

### Manufacturing of Packages

While injection stretch blow molding has proven to be a suitable manufacturer technique, other manufacturing techniques may be used. Various suppliers including, but not limited to, the Owens-Brockway Division of Owens-Illinois are capable of making packages of the present invention (e.g., specification number N-41701). In the formation of a plastic bottle formed using an Injection-Stretch-Blow-Molding (ISBM) molding process or an Injection Blow Molding (IBM) process, a semi-molten plastic tube is filled with pressurized air, thereby forcing the tube to expand outwardly to contact a mold surface in the shape of the desired container. Still another process, Injection Molding (IM), forms the container by forcing molten plastic into a mold in the desired container shape. While the use of injection blow molding (IBM) and injection stretch blow molding (ISBM) to mold clear plastic aerosol bottles has been documented, extrusion blow molding (EBM) could also be utilized for the packages of the present invention. This possibility has become a reality with the introduction of PETG and PCTG resins with increased melt strength. Materials with greater melt strength allow for the extrusion of thicker parisons and the production of thick walled bottles. In the case of optically clear bottles, possible resins include, but are not limited to, PETG and clarified polypropylene. In addition to these well known resin options, there are polyester/polycarbonate blends under development by Eastman for EBM applications. These blends provide chemical resistance and improved thermal resistance over PETG. Each of these processes, as well as other processes known to those skilled in the art, can be used to form the plastic packages of the present invention.

### Propellant/Pressurized Fluid

Several types of materials may be used to pressurize the container of the present invention. These materials include, but are not limited to, propellants and compressed gases. Propellants of the present invention include, but are not limited to, butane, isobutane, propane, dimethyl ether, 1, 1 difloroethane and mixtures thereof. Compressed gases of the present invention include, but are not limited to, nitrogen (N₂), carbon dioxide (CO₂), and mixtures thereof.

### EXAMPLES

The following examples illustrate the pressurized plastic containers of the present invention. Examples of the present invention are not intended to be limiting thereof:

### Example 1

The container following the steps in Table 2. Fill the bottle made of an 80/20 blend of PET/PC with 30.0 g (+/- 0.3g) concentrate of commercial body spray. Crimp on commercially available valve. Fill 20.0g (+/- 0.2g) propellant having a pressure of about 379.1 kPa (55 psi) into each bottle. Hot tank package to about 55°C for about 2 minutes. These packages were then subjected to the test methods outlined above in Table 2. All success criteria were met.

### Comparative Example

A PET material such as Eastman EN076^{™} when subjected to the steps in Table 1 will have a good to fair Δ_{haze} result. A PCTG/PC blend material such as Eastman DA510™ when subjected to the steps in Table 1 will have a very good to excellent Δ_{haze} result.

Eastman EN076^{™} when subjected to the steps in Table 2 is likely to fail one or more steps 4-6 as outlined in Table 2. Particularly, Eastman EN076^{™} is likely to have a Δ_{haze} of about 20% or more. Eastman DA510^{™}, however, when subjected to the steps in Table 2 is likely to pass all steps 4-6 as outlined in Table 2. Particularly, Eastman DA510^{™} is likely to have a Δ_{haze} of less than 20%.

## Claims

1. A plastic pressurized package having a hollow, plastic, non-round cross-section body, a sealing valve and an actuator, **characterized in that** the plastic of the body is a blend of a first polymer selected from the group consisting of polyesters, non-crystalline polyester copolymers and mixtures thereof, and a second polymer that is different from the first polymer and selected from the group consisting of polyamides, polycarbonates, polyacrylates, polycarbonate copolymers, polyesters, polyester copolymers and mixtures thereof, said first polymer being included at a ratio of greater than 70% in relation to said second polymer and optional additional materials, said plastic pressurized package being able to contain and dispense a pressurized fluid of at least 103.4 kPa greater than atmospheric pressure at 25°C.

2. The plastic pressurized package of claim 1 wherein said package has a wall thickness of from 0.65 mm to 3.25 mm.

3. The plastic pressurized package of any one of claims 1 to 2 wherein the first polymer is substantially amorphous non-crystalline polyethylene terephthalate or non-crystallizing polyethylene terephthalate.

4. The plastic pressurized package of any one of claims 1 to 3 wherein said package has a heat deflection temperature of at least 65°C under an applied load of 455.1 kPa.

5. The plastic pressurized package of any one of claims 1 to 4 wherein said package has a thermal resistance of at least 58°C.

6. The plastic pressurized package of any one of claims 1 to 5 wherein said package has an initial haze value of less than 10%.

7. The plastic pressurized package of any one of claims 1 to 6 wherein said package exhibits a high impact resistance of at least 1.83 m.

8. The plastic pressurized package of any one of claims 1 to 7 further comprising an additional material selected from the group consisting of colorants, fillers, additives, and mixtures thereof.

9. The plastic pressurized package of any one of claims 1 to 8 wherein said first polymer is a polyester copolymer selected from the group consisting of polyethylene terephthalate glycol-modified, polycyclohexanedimethanol terephthalate, polycyclohexanedimethanol terephthalate isophthalate, polycyclohexanedimethanol terephthalate glycol, and mixtures thereof, and the second polymer is a polycarbonate.

10. The plastic pressurized package of claim 1 wherein said first polymer is a non-crystalline polyester copolymer and is amorphous.

11. The plastic pressurized package of any one of claims 1 to 8, wherein the second polymer is polycarbonate.

12. The plastic pressurized package according to any of the preceding claims wherein the package is practiced as a product selected from antiperspirants, deodorants, hair products, household products, cooking sprays, beverages, perfumes, shaving creams/gels, or drug products.

13. The plastic pressurized package according to any of the preceding claims wherein the shape of the cross-section is square, rectangle, oval, star, heart, diamond, polygons, trapezoid, rhombus, or triangle.

14. The plastic pressurized package according to any of the preceding claims, containing propellant or compressed gas.

15. Use of the plastic pressurized package, according to any of the preceding claims, for containing a personal care product.

## Patentansprüche

1. Druckbeaufschlagte Kunststoffverpackung mit einem hohlen Kunststoffkörper mit nichtrundem Querschnitt, einem Abdichtventil und einem Betätigungselement, **dadurch gekennzeichnet, dass** der Kunststoff des Körpers eine Mischung eines ersten Polymers, das ausgewählt ist aus der Gruppe bestehend aus Polyestern, nicht kristallinen Polyestercopolymeren und Mischungen davon, und eines zweiten Polymers, das ein anderes als das erste Polymer ist und ausgewählt ist aus der Gruppe bestehend aus Polyamiden, Polycarbonaten, Polyacrylaten, Polycarbonatcopolymeren, Polyestern, Polyestercopolymeren und Mischungen davon, wobei das erste Polymer in einem Verhältnis von mehr als 70 % in Bezug auf das zweite Polymer enthalten sind, und fakultativen Zusatzmaterialien ist, wobei die dnickbeaufschlagte Kunststoffverpackung ein druckbeaufschlagtes Fluid von mindestens 103,4 kPa über Atmosphärendruck bei 25 °C aufnehmen und abgeben kann.

2. Druckbeaufschlagte Kunststoffverpackung nach Anspruch 1, wobei die Verpackung eine Wanddicke von 0,65 mm bis 3,25 mm aufweist.

3. Druckbeaufschlagte Kunststoffverpackung nach einem der Ansprüche 1 bis 2, wobei das erste Polymer im Wesentlichen amorphes nicht kristallines Polyethylenterephthalat oder nicht kristallisierendes Polyethylenterephthalat ist.

4. Druckbeaufschlagte Kunststoffverpackung nach einem der Ansprüche 1 bis 3, wobei die Verpackung unter einer aufgebrachten Last von 455,1 kPa eine Wärmeableitungstemperatur von mindestens 65 °C aufweist.

5. Druckbeaufschlagte Kunststoffverpackung nach einem der Ansprüche 1 bis 4, wobei die Verpackung einen Wärmewiderstand von mindestens 58 °C aufweist.

6. Dnickbeaufschlagte Kunststoffverpackung nach einem der Ansprüche 1 bis 5, wobei die Verpackung einen Trübungsausgangswert von weniger als 10 % aufweist.

7. Dnickbeaufschlagte Kunststoffverpackung nach einem der Ansprüche 1 bis 6, wobei die Verpackung eine hohe Schlagfestigkeit von mindestens 1,83 m aufweist.

8. Druckbeaufschlagte Kunststoffverpackung nach einem der Ansprüche 1 bis 7, ferner umfassend ein zusätzliches Material, das ausgewählt ist aus der Gruppe bestehend aus Farbstoffen, Füllstoffen, Zusatzstoffen und Mischungen davon.

9. Druckbeaufschlagte Kunststoffverpackung nach einem der Ansprüche 1 bis 8, wobei das erste Polymer ein Polyestercopolymer ist, das ausgewählt ist aus der Gruppe bestehend aus Polyethylenterephthalat, das mit Glycol modifiziert ist, Polycyclohexandimethanolterephthalat, Polycyclohexandimethanolterephthalatisophthalat, Polycyclohexandimethanolterephthalatglycol und Mischungen davon, und das zweite Polymer ein Polycarbonat ist.

10. Druckbeaufschlagte Kunststoffverpackung nach Anspruch 1, wobei das erste Polymer ein nicht kristallines Polyestercopolymer ist und amorph ist.

11. Druckbeaufschlagte Kunststoffverpackung nach einem der Ansprüche 1 bis 8, wobei das zweite Polymer Polycarbonat ist.

12. Druckbeaufschlagte Kunststoffverpackung nach einem der vorstehenden Ansprüche, wobei die Verpackung als ein Produkt ausgeführt ist, das ausgewählt ist aus schweißhemmenden Mitteln, Deodorants, Haarprodukten, Haushaltsprodukten, Kochsprays, Getränken, Duftstoffen, Rasiercremes/-gelen oder Arzneimittelprodukten.

13. Druckbeaufschlagte Kunststoffverpackung nach einem der vorstehenden Ansprüche, wobei die Form des Querschnitts quadratisch, rechteckig, oval, sternförmig, herzförmig, rautenförmig, polygonal, trapezförmig, rhombusförmig oder dreieckig ist.

14. Druckbeaufschlagte Kunststoffverpackung nach einem der vorstehenden Ansprüche, enthaltend ein Treibmittel oder komprimiertes Gas.

15. Verwendung der druckbeaufschlagten Kunststoffverpackung nach einem der vorstehenden Ansprüche zur Aufnahme eines Körperpflegeproduktes.

## Revendications

1. Conditionnement pressurisé en plastique possédant un corps creux en plastique, de coupe transversale non ronde, une soupape d'étanchéité et un actuateur, **caractérisé en ce que** le plastique du corps est un mélange d'un premier polymère choisi dans le groupe constitué de polyesters, copolymères de polyester non cristallins et leurs mélanges, et d'un deuxième polymère qui est différent du premier polymère et est choisi dans le groupe constitué de polyamides, polycarbonates, polyacrylates, copolymères de polycarbonate, polyesters, copolymères de polyester et leurs mélanges, ledit premier polymère étant inclus à un rapport supérieur à 70 % par rapport audit deuxième polymère et à des matériaux supplémentaires facultatifs, ledit conditionnement pressurisé en plastique pouvant contenir et distribuer un fluide sous une pression au moins 103,4 kPa supérieure à la pression atmosphérique à 25 °C.

2. Conditionnement pressurisé en plastique selon la revendication 1, dans lequel ledit conditionnement a une épaisseur de paroi allant de 0,65 mm à 3,25 mm.

3. Conditionnement pressurisé en plastique selon l'une quelconque des revendications 1 à 2, dans lequel le premier polymère est du polyéthylène téréphtalate non cristallin essentiellement amorphe ou du polyéthylène téréphtalate non susceptible de cristallisation.

4. Conditionnement pressurisé en plastique selon l'une quelconque des revendications 1 à 3, où ledit conditionnement a une température de déformation à la chaleur d'au moins 65 °C sous une charge appliquée de 455,1 kPa.

5. Conditionnement pressurisé en plastique selon l'une quelconque des revendications 1 à 4, où ledit conditionnement a une résistance thermique d'au moins 58 °C.

6. Conditionnement pressurisé en plastique selon l'une quelconque des revendications 1 à 5, où ledit conditionnement a une valeur initiale de trouble inférieure à 10 %.

7. Conditionnement pressurisé en plastique selon l'une quelconque des revendications 1 à 6, où ledit conditionnement présente une résistance élevée à l'impact d'au moins 1,83 m.

8. Conditionnement pressurisé en plastique selon l'une quelconque des revendications 1 à 7, comprenant en outre un matériau supplémentaire choisi dans le groupe constitué de colorants, charges, additifs et leurs mélanges.

9. Conditionnement pressurisé en plastique selon l'une quelconque des revendications 1 à 8, dans lequel ledit premier polymère est un copolymère de polyester choisi dans le groupe constitué de polyéthylène téréphtalate modifié par du glycol, polycyclohexanediméthanol téréphtalate, polycyclohexanediméthanol téréphtalate isophtalate, polycyclohexanediméthanol téréphtalate glycol et leurs mélanges, et le deuxième polymère est un polycarbonate.

10. Conditionnement pressurisé en plastique selon la revendication 1, dans lequel ledit premier polymère est un copolymère de polyester non cristallin et est amorphe.

11. Conditionnement pressurisé en plastique selon l'une quelconque des revendications 1 à 8, dans lequel le deuxième polymère est du polycarbonate.

12. Conditionnement pressurisé en plastique selon l'une quelconque des revendications précédentes, où le conditionnement est mis en pratique en tant que produit choisi parmi les anti-transpirants, les déodorants, les produits capillaires, les produits ménagers, les aérosols de cuisson, les boissons, les parfums, les crèmes/gels de rasage ou les produits médicamenteux.

13. Conditionnement pressurisé en plastique selon l'une quelconque des revendications précédentes, dans lequel la forme de la coupe transversale est un carré, un rectangle, un ovale, une étoile, un coeur, un losange, des polygones, un trapèze, un losange, ou un triangle.

14. Conditionnement pressurisé en plastique selon l'une quelconque des revendications précédentes, contenant un propulseur ou un gaz comprimé.

15. Utilisation du conditionnement pressurisé en plastique, selon l'une quelconque des revendications précédentes, pour contenir un produit de soins d'hygiène personnelle.
